

Dec. 3, 1935.

G. J. EASTER

2,023,044

CORE FOR AND METHOD OF PRODUCING HOLLOW REFRACTORIES

Filed Dec. 18, 1933

*Fig. 1.*



*Fig. 2.*



INVENTOR.  
GEORGE J. EASTER

BY

*R.C. Bemner*

ATTORNEY.

## UNITED STATES PATENT OFFICE

2,023,044

CORE FOR AND METHOD OF PRODUCING  
HOLLOW REFRACTORIESGeorge J. Easter, Niagara Falls, N. Y., assignor  
to The Carborundum Company, Niagara Falls,  
N. Y., a corporation of Pennsylvania

Application December 18, 1933, Serial No. 702,941

9 Claims. (Cl. 49—79)

This invention relates to a new method for the manufacture of nonmetallic articles made by casting molten material into refractory molds containing one or more cores for the fabrication of articles with recesses, holes, etc. Such articles are often found to contain cracks when delivered from the molds, this cracking being caused by the thermal inflexibility of the core which sets up internal stresses in the cast article as it cools about the inclosed core.

I have discovered that if the core is made of material of higher thermal expansion than the material being cast, and if the heat capacity of the core be kept low both by keeping the amount of material low and by using material whose inherent specific heat is low, the core rapidly reaches a maximum temperature and size when the molten material is poured around it; and then after the walls of the casting solidify, it shrinks away from the shell of cast material. Due to its higher thermal expansion, the core shrinks faster than the casting even though air is excluded from the core. In this manner, as the article is being formed within the mold the amount of internal stress is minimized and the article as finally made is free of cracks.

My invention is illustrated in the drawing in which

Figure 1 is a vertical cross-section through the mold with the core in place ready for the casting operation; and

Figure 2 shows diagrammatically one method of applying my invention to the manufacture of crucibles of cast alumina or of similar refractory material.

The core in a typical case, such as making a casting of fused alumina, is made of chromite or magnesia both of which have appreciably higher coefficients of expansion than alumina. In Figure 1, the walls 3 of the mold are made of material sufficiently refractory to contain the molten material of the casting without destruction or disintegration of the mold walls. The mold is provided with a riser 4 of ample size to permit complete filling of the mold without interference by material freezing in the header 5. The riser is preferably made wedge shaped with its minimum section immediately adjacent the mold, so that removal of the excess material constituting the header 5 is facilitated. The walls of the core 6 are in general, as is indicated, relatively thin and exposed to the air on one side. The air space within such a core may be a dead air space, so as not to hasten the cooling of the core. In special cases, I may use as core material refractory alloys

of chromium and iron, and chromium, iron and nickel; but when these are used the interior of the core must be air cooled as the core is not so refractory as the casting and any melting of the core is to be avoided. Such metal cores are in particular useful when materials such as chromite which have in themselves high thermal expansion coefficients are being cast.

In some cases I have found it advantageous to overlay the core with a layer 7 of blotting paper 10 or other destroyable carbonaceous material against which the molten material will initially come in contact.

Should it be desirable, as above referred to, to air cool the core, this may be accomplished as indicated diagrammatically in Figure 2. The core may be shaped as required by the form of recess which the desired article is to have. In accordance with Figure 2, a trough shaped refractory piece is to be cast in the mold 3a by the use of a 20 core 6a. Cooling air is supplied to the interior of the core by the inlet 9 and the heated air discharged by way of the outlet 10 or out at the ends of the trough.

Cores utilizing the method of this invention may be made of ceramically bonded and burned or temporarily bonded granular material. The cores may be either monolithic or may be made up in sections. For example, I have built up cores from slabs made by bonding chromite grain with sulfite 30 pitch, the slabs being assembled into a hollow shaped core for the manufacturing of crucibles with rectangular openings. Furthermore, the core may be precast, either as a single casting, or in sections. When precast, ceramically bonded 35 or metallic cores are used, the cores may be used repeatedly until worn or warped, and even then may be patched or straightened for additional use. The essential requirement is that the refractory material of the core have a higher coefficient of 40 expansion than the material being cast. The use of chromite cores is particularly advantageous in that the material is highly refractory and yet completely inert, so that no reaction takes place between the core and the molten casting.

The mold proper may, for example, be made of bonded refractory granular material according to regular molding practice as adapted to the casting of refractory non-metallic fusions. The core should be interlocked with the mold to prevent displacement by the material being cast 50 using any suitable means not shown other than to indicate the core set in a close fitting groove around its base.

In accordance with my invention, I provide

a core which will quickly become heated to its maximum temperature so that it will attain its maximum size before the cast shell next to it completely solidifies. In cooling down, the core 5 will shrink faster than the casting so that strains will not be set up which will break the casting. The layer of paper or other carbonaceous material has the advantage of imparting a further degree of flexibility between the core and the 10 casting, and reducing the thermal shock to the core in that it allows additional time for the heating of the core before the cast face solidifies in contact with it. The layer of paper may be omitted successfully in many cases however.

15 While I have explained in detail the manner of performing my invention as illustrated by certain specific embodiments, it will be understood that my invention is not limited to the specific details of these embodiments, but may be otherwise embodied and practiced within the scope 20 of the following claims.

I claim:

1. In combination with a mold for casting low refractories, a core of low thermal capacity 25 and having a higher coefficient of thermal expansion than the material being cast.
2. In a mold for fabricating cast non-metallic articles, a core whose coefficient of thermal expansion is greater than that of the material being cast.
3. The method of forming refractory castings with openings or recesses comprising casting the molten alumina in a mold including a core having thin walls of chromite.

4. The method of forming refractory castings with openings or recesses comprising casting the molten alumina in a mold including a core having thin walls of fused magnesia.

5. The method of forming chromite castings 5 with openings or recesses comprising casting the molten chromite in a mold provided with a core having thin walls of a ferro-chromium alloy.

6. In combination with a mold for forming cast non-metallic articles, a hollow core having 10 thin walls whose coefficient of thermal expansion is greater than that of the material being cast.

7. The method of forming refractory castings with openings or recesses comprising casting the molten refractory material in a mold including 15 a hollow core and passing cooling fluid through the hollow core to prevent overheating of the core during casting.

8. The method of forming refractory castings with openings or recesses comprising casting mol- 20 ten material in a mold including a hollow core formed of material having a lower freezing point than the temperature of the molten material being cast and passing cooling fluid through the hollow core.

9. In the process of casting molten non-me- 25 tallic refractory materials the steps which comprise shaping the molten material by casting it against a refractory wall, permitting heat to escape through said wall and governing the tem- 30 perature of said wall by circulation of a cooling fluid in contact therewith but out of contact with the cast material.

GEORGE J. EASTER.